

## UNITED STATES PATENT OFFICE

2,313,523

## PHOTOGRAPHIC MATERIAL

Thomas S. Donovan and Walter V. Wadman,  
Rochester, N. Y., assignors to Eastman Kodak  
Company, Rochester, N. Y., a corporation of  
New Jersey

No Drawing. Application June 18, 1940,  
Serial No. 341,182

9 Claims. (Cl. 95—88)

This invention relates to photographic agents, and particularly photographic developers in dry form or compositions in dry form adapted to be added to solutions suitable for developing photographic paper and film.

It is known to add formaldehyde to developers in order to harden the gelatin or the colloidal layer in which the silver halide is dispersed. It is also added in order to obtain high contrast. Formaldehyde is a gas at ordinary temperatures and when added as such to developer, it must be added at the time the developer is prepared. Paraformaldehyde, a polymer of formaldehyde, has been used instead of formaldehyde for these purposes. It has been added to the aqueous solutions of the developers and it has also been proposed that it be mixed with the solid components of the developer. However, paraformaldehyde has many properties which make it objectionable for use in this manner. It has a low solubility so that it is difficult to get it thoroughly dissolved in the aqueous developer. It polymerizes on standing to polymers of even lower solubility and from which the formaldehyde is not as easily utilized. It has a strong irritating odor characteristic of formaldehyde and it volatilizes to a certain extent in dry form to lose a part of its formaldehyde content.

This invention has for its object to provide a solid photographic composition which will yield an aldehyde such as formaldehyde when in aqueous solution and which is substantially free of the above difficulties. Another object is to provide a photographic composition of matter in dry form which is readily soluble in cold water and, when dissolved in aqueous solution in the presence of a base, will yield an aldehyde, the dry powder being substantially free of odor due to formaldehyde. Another object is to provide a composition of matter in dry form which contains formaldehyde in chemical combination so that it does not substantially volatilize and which is in such chemical condition that it will readily dissolve in water. Another object is to provide a packaged dry or solid developer containing an aldehyde or formaldehyde compound which will be released on solution and which can be sold in dry condition. Other objects are to improve the state of the art.

These and other objects are accomplished in accordance with our invention which includes a dry or solid mixture of a photographic agent and a compound of an aldehyde with a bisulphite. We have discovered that when this mixture is dissolved in water in the presence of a base, the aldehyde-bisulphite compound is decomposed to release aldehyde in the solution. At the same

time, sulphite is released in the photographic solution where it acts to protect against oxidation in known manner.

The solid mixture may contain the well-known materials which act to improve the action of photographic solutions. For instance, boric acid may be added thereto for its advantageous effect on the developed film or paper. Potassium bromide may be added. Water soluble compounds to restrict the swelling of gelatine or the like such as citrates, sulphates and phosphates may likewise be added thereto in solid condition. Fog restraining and inhibiting substances may be present.

15 The solid components including the developing agent and the aldehyde-bisulphite compound are mixed together in suitable proportions and then may be packaged for commercial distribution. It is undesirable to add a base to the dry developer since it would accelerate oxidation or deterioration of the developing agent. Also, the base in the presence of moisture would cause decomposition of the aldehyde-bisulphite salts with loss of the aldehyde. The base can be included in a separate package or may be added to the solution at the time it is prepared.

Our new composition of matter forms the developing solution when added to water in the presence of a base. The base reacts with the 30 aldehyde-sulphite mixture causing it to decompose into an aldehyde and sulphite. For instance, when sodium hydroxide is the base and sodium bisulphite is combined with formaldehyde, the reaction is as follows:



This action takes place only when the compound is in the presence of a base so that substantially no loss of formaldehyde takes place in the solid mixture until it is actually used. For the same reason the composition of matter does not have an odor of formaldehyde as is the case with the formaldehyde yielding substances heretofore employed. Strong inorganic bases such as sodium hydroxide, sodium carbonate, etc., increase the rate of aldehyde formation and are preferred. They are also preferred for the reason that they increase contrast.

The aldehyde may be combined with alkali metal bisulphites such as sodium and potassium bisulphites.

The invention is of particular value in connection with phenol type developers such as hydroquinone, ortho catechol para-aminophenol and its salts, monomethyl para-aminophenol sulfate and chlorhydroquinone.

While we have described our invention as being particularly valuable for preparing developing compositions, it is applicable to the preparation of solid compositions which upon dissolving in water yield solutions which affect a photographic image. For instance the solid preparation may comprise the aldehyde-bisulfite compound and an intensifying agent. Although formaldehyde is preferred, other aldehydes such as acetaldehyde can be combined with the bisulfite. Water soluble aldehydes are best for aqueous developers.

In the following examples, which illustrate the method of compounding the compositions of matter and preparing developing solutions, we have given examples of how the dry compound is added to the developing solution in the presence of a base. However, our invention applies only to the solid material containing the developer and formaldehyde-bisulfite mixture and does not cover the aqueous solution or the base contained therein.

*Example 1*

A solid granular mixture is prepared from the following:

|                                      | Grams |
|--------------------------------------|-------|
| Sodium bisulfite                     | 1.90  |
| CH <sub>2</sub> O-NaHSO <sub>3</sub> | 37.00 |
| Boric acid                           | 7.50  |
| Hydroquinone                         | 22.50 |
| Potassium bromide                    | 1.57  |

This mixture can be packaged and will keep without loss for a long period of time. To prepare a developing solution it may be added to 9.50 grams of sodium hydroxide and water added to make one liter. This developing formula is superior in all respects to those in which paraformaldehyde has heretofore been employed. The solid material readily dissolves and has no odor.

*Example 2*

A solid granular or powdered mixture is prepared from the following:

|                                      | Grams |
|--------------------------------------|-------|
| Sodium bisulfite                     | 1.90  |
| CH <sub>2</sub> O-NaHSO <sub>3</sub> | 37.00 |
| Boric acid                           | 7.50  |
| Hydroquinone                         | 22.5  |
| Potassium bromide                    | 1.57  |

To prepare a developing solution from this composition it is added to 27.70 grams sodium carbonate in aqueous solution and water is added to make one liter.

*Example 3*

|                                      | Grams |
|--------------------------------------|-------|
| Sodium bisulfite                     | 2.18  |
| CH <sub>2</sub> O-NaHSO <sub>3</sub> | 41.8  |
| Boric acid                           | 8.5   |
| Hydroquinone                         | 25.6  |
| Potassium bromide                    | 1.78  |

To prepare a developing solution from this solid mixture it is added in the proportions given to a solution of 10.04 grams sodium hydroxide. Water is added to make one liter.

*Example 4*

A solid powdered mixture of the following is prepared:

|                               | Grams |
|-------------------------------|-------|
| Sodium bisulfite              | 2.18  |
| Acetaldehyde-sodium bisulfite | 46.9  |
| Boric acid                    | 8.5   |
| Hydroquinone                  | 25.6  |
| Potassium bromide             | 1.78  |

To prepare a developing solution the foregoing mixture and 10.44 grams of sodium hydroxide are added to water to make one liter of solution.

Our invention has the particular advantage that developers containing aldehydes and particularly formaldehyde can be quickly prepared in a simple manner without the disadvantage of extra manipulations such as adding formaldehyde or dissolving paraformaldehyde. It has great solubility, substantially no odor and a long exhaustion life. It has the outstanding advantage that sodium sulphite or equivalent materials need not be added. However, it is to be understood that such materials may be present, if desired.

What we claim is:

1. A composition of matter in solid or powder form, adapted to form a photographic solution containing free aldehyde in quantities sufficient to act as a hardener and a sulphite when dissolved in water in the presence of a base, comprising a photographic agent which will affect a photographic image and a compound of an aldehyde with a bisulfite.

2. A composition of matter in solid or powder form, adapted to form a developing solution containing free aldehyde in quantities sufficient to act as a hardener and a sulfite when dissolved in water in the presence of a base, comprising a photographic developing agent and a compound of an aldehyde with a bisulfite.

3. A composition of matter in solid or powder form adapted to form a developing solution containing a free aldehyde in quantities sufficient to act as a hardened and a sulfite when dissolved in water in the presence of a base, comprising a phenolic developing agent and a compound of an aldehyde with a bisulfite.

4. A packaged composition of matter in solid or powder form which is stable over extended periods of time and which is adapted to form a developing solution containing free formaldehyde in quantities sufficient to act as a hardener and a sulphite when dissolved in water in the presence of a base, comprising a photographic developing agent and a compound of formaldehyde with an alkali metal bisulfite.

5. A composition of matter in solid or powder form adapted to form a developing solution containing free formaldehyde in quantities sufficient to act as a hardener and a sulphite when dissolved in water in the presence of a strong inorganic base, comprising a photographic developing agent and a compound of formaldehyde with an alkali metal bisulfite.

6. A composition of matter in solid or powder form, adapted to form a developing solution containing free formaldehyde in quantities sufficient to act as a hardener and a sulphite when dissolved in water in the presence of a base, comprising a phenolic developing agent and a compound of formaldehyde with a bisulfite.

7. A composition of matter in solid or powder form adapted to form a developing solution containing free formaldehyde in quantities sufficient to act as a hardener and a sulphite when dissolved in water, in the presence of a strong inorganic base, comprising a phenolic developing agent and a compound of formaldehyde with an alkali metal bisulfite.

8. A composition of matter in solid or powder form adapted to form a developing solution containing free formaldehyde in quantities sufficient to act as a hardener and a sulphite when

dissolved in water, in the presence of a strong inorganic base, comprising hydroquinone and  $\text{CH}_2\text{O.NaHSO}_3$ .

9. A packaged composition of matter in solid or powder form which is stable over extended periods of time and which is adapted to form a developing solution containing an aldehyde and

a sulphite when dissolved in water in the presence of a base, comprising a photographic developing agent and a compound of an aldehyde with an alkali metal bisulphite.

5

THOMAS S. DONOVAN.  
WALTER V. WADMAN.